

(No Model.)

J. G. BEALE.

MANUFACTURE OF PLANISHED STEEL SHEETS.

No. 364,568.

Patented June 7, 1887.

*Fig. 1.*



*Fig. 2.*



WITNESSES:

*F. G. Gaither,  
A. H. Whittelsey*

INVENTOR,

*Joseph G. Beale,  
Darwin S. Wolcott*

At'ty.

# UNITED STATES PATENT OFFICE.

JOSEPH G. BEALE, OF LEECHBURG, PENNSYLVANIA.

## MANUFACTURE OF PLANISHED STEEL SHEETS.

SPECIFICATION forming part of Letters Patent No. 364,568, dated June 7, 1887.

Application filed February 10, 1887. Serial No. 227,103. (No model.)

*To all whom it may concern:*

Be it known that I, JOSEPH G. BEALE, residing at Leechburg, in the county of Armstrong and State of Pennsylvania, a citizen of the United States, have invented or discovered certain new and useful Improvements in the Manufacture of Planished Steel Sheets, of which improvements the following is a specification.

10 In the accompanying drawings, which make part of this specification, Figure 1 is a plan view of a steel sheet, showing the sheet in one of the preliminary stages of its manufacture. Fig. 2 is a transverse sectional view showing a 15 number of the sheets shown in Fig. 1 arranged in a pack.

In manufacturing planished sheet-iron the sheets, after being rolled to approximately the desired gage, are scaled by an acid bath or other 20 suitable means, and then the oxide which immediately forms on the surfaces of the sheets after the removal of the scale is "revived" by heating the plates to a cherry-red in the presence of or in contact with some suitable carbonaceous or other deoxidizing material. After 25 the oxide surface has been revived in the manner above stated, the sheets are then hammered in packs, thereby reducing them to the desired gage and producing a smooth, polished, and 30 non-oxidizable surface. This method of treatment or working has been attempted on sheets of steel, but has been found impracticable, for the reason that the additional carbon taken up by the steel sheets during the "reviving" 35 operation above described renders the steel very hard and brittle, and therefore useless for subsequent working into articles of manufacture.

The object of the invention herein is to so 40 treat steel sheets as to not only produce a smooth and polished surface, but also to render it softer and even more pliable in working than steel sheets of same gage which have not been subjected to my improved method.

45 In the practice of my invention the sheets, which are of mild or low carbon steel, are rolled in the usual manner down to twenty-wire gage, or less. These sheets, on which a thin coating of oxide has formed during the 50 rolling operation, are then placed in packs of fifty (more or less) in a suitable oven and heated

to such a degree—*i. e.*, a cherry-red—that the oxygen of the surface coating will combine with the carbon of the body of the sheets, and thereby revivify such coating either entirely 55 or to a considerable extent, and at the same time reduce the carbon in the sheets to an equal extent, and thereby render the same softer and more easily worked. After being heated as above described, the sheets are 60 placed under a hammer, the integrity of the packs being preserved, and are hammered until cold, as is the usual practice in planishing sheets.

As the sheets of the pack are liable to stick 65 together when hammered unless great care is exercised in the heating of the packs, I propose to pass the sheets, either heated or cold, and before their surface coating has been revivified, between rolls having shallow recesses 70 or indentures formed in their operative faces in any suitable manner. The sheets 1 so rolled will have a large number of small nodules or elevations, 2, on their surfaces, formed by the forcing of portions of the sheets into the recesses or indentures in the rolls during the 75 rolling operation. The sheets of steel thus prepared are arranged in packs of fifty, the number of sheets being increased or decreased as circumstances may dictate. The packs are 80 placed in a suitable furnace, heated to the proper temperature, as above described, and finally hammered. When arranged in packs, the sheets are held apart by the nodules or projections 2, thereby permitting of a com- 85 paratively free circulation of the heat through the pack, and consequently avoiding an undue heating of the external sheets. In addition to uniformity in heating consequent upon the separation of the sheets, as above stated, 90 these nodules form supports to the sheets, and hence allow of a certain resilient action on the part of the sheets when struck by the hammer, causing them to spring apart at each upward movement of the hammer, thereby avoiding 95 all liability to the sheets being welded or stuck together by the operation of the hammer. The welding or sticking together is further prevented by the air between the separate sheets, forming a sort of cushion, as it were, between them.

As there is a greater body of good—*i. e.*, non-

oxidized—metal under the oxide covering of each nodule than there is under the oxide coating of the level portions of the sheet, and the oxide coating of the nodules will therefore be 5 revivified to a greater extent than the coatings of the other portions, the location of the nodules will be indicated in the finished sheets by comparatively light-colored spots, shading off into the darker color of the other portions 10 of the sheets, which impart a rich mottled effect to the sheets.

The revivifying action does not extend entirely through the oxide coating, but is conducted to such an extent as to firmly unite a 15 thin oxide film to the surface of the sheets, which will not crack or break loose when the sheet is bent or otherwise worked.

I claim herein as my invention—

1. The herein-described method of planishing steel sheets, which consists in heating the 20

sheets to such a temperature as will permit the carbon in the sheets to act on the oxide of the surface coating, thereby reviving such surface coating, and then hammering the sheets, substantially as set forth.

25

2. The herein-described method of planishing steel sheets, which consists in forming nodules or projections on the surface of the sheets, then heating the sheets to such a temperature as will permit the carbon therein to 30 act upon the oxide of the surface coating, thereby reviving such surface coating, and finally hammering the sheets, substantially as set forth.

In testimony whereof I have hereunto set my hand.

JOSEPH G. BEALE.

Witnesses:

DARWIN S. WOLCOTT,  
R. H. WHITTLESEY.